

April 3, 1945.

C. E. BINNS ET AL

2,372,878

INSULATING SHEET OR STRIP

Filed Nov. 16, 1942



Inventors:  
Charles Edward Binns,  
Stanley Palmer,  
by Pierce & Scheffler,  
Attorneys.

## UNITED STATES PATENT OFFICE

2,372,878

## INSULATING SHEET OR STRIP

Charles Edward Binns and Stanley Palmer, Liversedge, England, assignors to Versil Limited, Liversedge, England, a company of Great Britain and Northern Ireland

Application November 16, 1942, Serial No. 465,794  
In Great Britain September 23, 1942

1 Claim. (Cl. 154—2.6)

This invention relates to insulating sheets or strips of the kind which are made from glass silk.

Previously, such a sheet was formed by winding layers of glass silk fibres onto a drum and subsequently applying varnish to one side of the glass silk sheet so formed. Any attempt to varnish this sheet in the normal way, that is to say by dipping and baking, caused the sheet to shrink in the weft direction.

According to this invention both sides of the sheet or strip are varnished. The method consists of pre-varnishing the drum, applying a layer or layers of glass silk, re-varnishing the drum over the silk and finally baking and removing the silk sheet from the drum. Alternatively, the sheet can be cut into strips before removing it from the drum, the silk being thus removed in the form of a tape.

One form of apparatus for carrying out the present invention is illustrated in the accompanying drawing, wherein:

Fig. 1 is a side elevation;

Fig. 2 is a front view of the drum shown in Fig. 1 on which a sheet has been formed, part of the said sheet being removed to show the layers of lubricant, varnish, and glass silk.

Fig. 3 shows a short length of tape made on the apparatus illustrated in Fig. 1, the layers of the tape being separated to show its construction.

Referring to the drawing:

A glass furnace 2 and associated spinning bar 3 are arranged above a drum 4 adapted to revolve about a horizontal axis and provided with means for driving it at the desired speed or speeds. As shown the drum is carried by a shaft 5 which is supported in bearings 6 mounted on the framework 7 and is driven by a motor 8, pulleys 9, 10 and a belt 11. The glass filaments 12 issuing from the furnace through the spinning bar are guided by a pair of pins 13. The guide is carried by an endless band 14 running on rollers or

pulleys 15 across the width of the drum so as to be traversed to and fro by the motor 16 through the gear box 17. An eye or other guiding or grouping device or a single inclined pin may be employed instead of the pins 15 if desired.

For the cutting operation, a wheel type cutter 18 is traversed across the face of the drum at the requisite speed by any of the usual forms of traversing gear.

10 In the apparatus illustrated, a movable guide 13 is shown. However, if desired, the guide may be fixed and a movable furnace provided. The drum surface 4 is first lubricated and the lubricant *a* is allowed to set. The varnish *b* is then sprayed on to the drum surface 4 and a layer or layers of glass silk *c* is then wound on to the drum. When sufficient silk *c* has been wound more varnish *d* is sprayed on and the whole sheet is baked. The silk is then cut off in sheet or tape form.

15 This method results in a material with a coat of varnish on each side of the glass fibres, having an apparent density of more than 20 lbs. per cubic foot. The advantages of the material are as follows:

- 20 1. It has a greater strength in the weft direction.
2. A higher di-electric strength.
3. A greater resistance to moisture, and
4. An improved surface appearance.

25 What we claim and desire to secure by Letters Patent is:

Method for making an insulating material which consists in forming a sleeve on a drum by 30 first lubricating the drum, prevarnishing the drum, spinning a layer of substantially parallel glass silk fibers on the drum, revarnishing the drum over the silk and baking whilst on the drum and then removing the material from the drum 35 by cutting the sleeve to the desired form.

CHARLES EDWARD BINNS.  
STANLEY PALMER.